

S. CORNELL.

APPARATUS AND PROCESS FOR PREPARING PULVEROUS IRON ORES AND THE LIKE FOR SMELTING IN BLAST FURNACES AND USE IN OPEN HEARTH FURNACES.

APPLICATION FILED FEB. 9, 1909.

962,006.

Patented June 21, 1910.



Figure 2.



*WITNESSES:*

WITNESSES:

INVENTOR.

*Sidney Cornell*

S. CORNELL.

APPARATUS AND PROCESS FOR PREPARING PULVEROUS IRON ORES AND THE LIKE FOR  
SMELTING IN BLAST FURNACES AND USE IN OPEN HEARTH FURNACES.

APPLICATION FILED FEB. 9, 1909.

962,006.

Patented June 21, 1910.

2 SHEETS—SHEET 2.

Figure 3.



WITNESSES:

W. C. Reed  
H. J. Black.

INVENTOR.

Sidney Cornell.

# UNITED STATES PATENT OFFICE.

SIDNEY CORNELL, OF DUQUESNE, PENNSYLVANIA.

## APPARATUS AND PROCESS FOR PREPARING PULVEROUS IRON ORES AND THE LIKE FOR SMELTING IN BLAST-FURNACES AND USE IN OPEN-HEARTH FURNACES.

962,006.

Specification of Letters Patent. Patented June 21, 1910.

Application filed February 9, 1909. Serial No. 476,891.

*To all whom it may concern:*

Be it known that I, SIDNEY CORNELL, a citizen of the United States, residing at Duquesne, county of Allegheny, and State 5 of Pennsylvania, have invented certain new and useful Improvements in Apparatus and Processes for Preparing Pulverous Iron Ores and the Like for Smelting in Blast-Furnaces and Use in Open-Heart Furnaces, 10 of which the following is a specification.

My invention relates to means for sintering and otherwise preparing pulverous iron ores, flue dust, magnetic concentrates, and other materials of similar nature for smelting 15 in blast furnaces and use in open heart furnaces used in the manufacture of iron and steel. Such materials being naturally in a state of too fine division or composed of too small particles to be retained in those 20 furnaces while subjected to blast in smelting, resort has been had to sintering and briquetting them into workable conditions.

Pulverous iron ores, flue-dust, or magnetic 25 concentrates may, without admixture with other material, be sintered or clinkered by heating them to a temperature slightly above 2500 degrees Fahrenheit, such action being caused by the melting of a part of the material so heated, and said fused portion acting 30 as a binder for the unfused residue of material. This action is probably due to the formation of ferrous silicates which constitute the binder of the residue of the material remaining unsintered, the sintering process, 35 thus making its reduction more difficult and costly, and it is, therefore, desirable that it be returned to the ferric condition by subjecting the clinker while heated to oxidation in order to its being more easily smelted. 40 if used in a blast furnace, and becoming a more efficient material in open heart furnaces because of the larger content of oxygen in the oxidized clinker, than in the un-oxidized clinker.

My invention has for its object a single 45 simple apparatus, and a continuous process for sintering these pulverous materials, restoring them to the ferric condition, and delivering them in masses of convenient size 50 for handling and working.

My apparatus is shown in the accompanying drawings, forming a part of this specification, and in which—

Figure 1 is a vertical longitudinal mid-section view of the construction; Fig. 2 is

a vertical cross-section view thereof taken on the line 2—2 in Fig. 1; and Fig. 3 is a perspective view thereof showing the walls of the apparatus partially broken away to disclose the interior arrangements. 60

The outer wall, 1, of the furnace is arched throughout its length, as shown. Within said outer wall, and spaced therefrom to form an intermediate chamber, is a second arched or curved wall, 2, 2<sup>1</sup>, which is broken at its crown by the longitudinal pit, 3. The walls 1, 2, 2<sup>1</sup>, are constructed of suitable refractory material to withstand high heat. 65

4, 4 are gas ducts bordering each side of the outer wall, 1, throughout its length, or nearly so; and opening from said ducts through said outer wall into the chamber 5, are the tubes or burners 6, 6. Apertures 7, 7, are formed in the crown of the outer wall 1, which opens into a smoke-box 8, connecting at its end with the stack 9, and opening into it; said arrangements being provided to enable the escape from the chamber 5 of the products of combustion. Below the chamber 5 are inclined tables or surfaces, 10, 11, arranged to receive from the chamber 5 the partially treated materials. Near the bottom of the pit, 3, and throughout its length lies a screw conveyer, 12, which is actuated through the gear, 13, or by any equivalent means for conveying power to rotate the same. At the outer end of said screw is placed the hopper 14. The screw conveyer, 12, in that part of its structure near the outer end thereof has the pitch of 80 its blade formed at an angle in which the conveying principle predominates, while the remainder and greater part of the blade is pitched at an angle in which the lifting principle predominates. 85 90 95

The operation of my construction and the consequent process are as follows:—The material to be treated is fed into the hopper, 14, and is forced into the pit, 3, by the conveyer, 12, which is rotated by power applied to the gear, 13. The material is continuously forced into the pit until the pit is filled from end to end and the material is forced above the upper edges of the pit and passes out and over upon the upper faces 100 of the curved walls 2, 2<sup>1</sup>. The gas passing through the ducts, 4, 4, and burners 6, 6, being ignited at the inner ends of the burners, heats the inside of the arched wall, 1, to a high degree, and the mass of 105 110

material being treated is heated directly and by the heat reflected from said arched wall. This induces a sintering of the outer portion of the material which becomes incrusted 5 with clinker. As more of the material is forced by the screw into and up through and out of the pit, 3, it rises with a wave-like motion (indicated by the dotted line 15 in Fig. 1), and breaks the crust or clinker 10 formed upon the upper face of the pile of material, turning or folding over the broken pieces of the crust, and exposing to the direct action of the heat the raw or unsintered side thereof, so that it becomes sintered 15 on all sides. As the feeding process continues the broken clinker piles up upon the curved walls, 2, 2<sup>1</sup>, beyond the angle of repose (indicated by the dotted line 16 in Fig. 2), and then rolls down upon the tables 20 10, 11. When it reaches these tables the material consists of conglomerated iron oxids, but a large portion of which is in ferrous or deoxidized condition. On these tables the broken clinker remains sufficiently 25 long for the air passing from below, through and over it into the chamber, 5, to oxidize the ferrous oxid of the clinker into ferric condition, whereby the material becomes properly prepared and workable in the 30 smelting furnace. When the clinker has laid long enough upon the tables to become sufficiently cool it is dumped into the car, 17, below. The air passing over the clinker on the inclined tables, cools the clinker, and 35 is at the same time highly heated thereby, and while aiding the combustion of the gas passing from the burners also aids in the production of a higher temperature within the furnace. The wavy motion given the 40 mass of material in the pit, 3, by the screw conveyer not only causes the breaking up of the crust or clinker formed upon the top of the pile of material, but also loosens and agitates the material beneath the crust, 45 thereby allowing any gases generated in the mass of material in the pit to escape through the breaks or rifts in the crust, while, in the treatment of flue dust it permits the elimination of the coke in the dust by the 50 burning out of this carbon, the products of combustion passing off through the smoke box and stack. The rate of clinkering can be controlled through the motion of the screw, and by regulating the speed of its 55 rotation, the maximum amount of material can be run through the apparatus consistent with proper treatment.

By the described apparatus and process I procure the formation of the pulverous materials treated in masses of size and weight available for smelting in blast furnaces and use in open hearth furnaces, and restore the deoxidized parts thereof to the ferric condition by a single continuous operation economically, rapidly and effectively conducted.

Having thus described my invention I claim:

1. In apparatus for sintering pulverous iron ores and the like, a heating chamber; means for producing flame in said chamber, 70 and means for conveying into said chamber material to be treated therein, and for breaking and discharging from said chamber the sintered portion of said material.

2. In apparatus for sintering pulverous iron ores and the like, a heating chamber; means for producing flame in said chamber; means for conveying material to be treated into said chamber, fracturing the sintered portion thereof when formed, and discharging it from said chamber, and means whereby said sintered product is arrested and exposed to the air while hot.

3. In apparatus for sintering pulverous iron ores and the like, a heating chamber; 85 means for producing flame in said chamber; means for conveying material to be treated into said chamber, exposing it in bulk to the heat therein, fracturing the sintered crust thereon when formed, and discharging said sintered crust from said chamber, and means for arresting and detaining said sintered product while hot to a current of air directed to said heating chamber.

4. The process of agglomerating pulverous iron ores and the like, which consists in subjecting the treated material in bulk to a high heat; converting the surface of the material exposed to such heat into a crust and fracturing said crust.

5. The process of treating pulverous iron ores and the like, which consists in subjecting the treated material in bulk to a high heat; converting the surface of the material exposed to such heat into a crust, and fracturing such crust and exposing it to the air while hot.

6. In apparatus for preparing pulverous iron ores and the like for smelting in blast furnaces or use in open hearth furnaces, the 110 combination of a heating chamber having an inclined floor; a channel opening to said floor; a screw conveyer lying within said channel and having a blade or blades of varied pitch, the pitch of said blade or 115 blades in the forward part of said conveyer having a pitch in which the conveying principle predominates, and the remainder or greater part of said blade or blades having a pitch in which the lifting principle predominates; a receptacle located in a lower plane than said inclined floor and adjacent thereto, a passage between said inclined floor and said receptacle, leading from the outer air to the interior of said heating 125 chamber; means for operating said conveyer, and means for heating the interior of said chamber.

7. In apparatus for preparing pulverous iron ores and the like for smelting in blast 130

furnaces or use in open hearth furnaces, the combination of a heating chamber having an arched roof and an inclined floor, a channel in said floor and a screw conveyer lying within said channel; a table located below the level of the floor of said chamber and at one side thereof; a passage over said table and opening into said heating chamber, and means for heating the interior of said chamber.

8. In apparatus for preparing pulverous iron ores and the like for smelting in blast furnaces or use in open hearth furnaces, the combination of a heating chamber, having an arched roof and arched floor; a channel opening through said floor; a screw conveyer lying within said channel and having a blade or blades of varied pitch, whereby said conveyer is adapted for conveying and lifting the material in which it rotates; a plurality of tables located below the level of the floor of said chamber and at the sides thereof; passages opening from said chamber and continuing past said tables; and means for the escape from said chamber of the products of combustion.

9. The process of preparing pulverous iron ores and the like for smelting in blast furnaces, or use in open hearth furnaces, consisting in first subjecting the material to a high heat and converting it into a conglomerated mass through the reduction of the ore as it exists in the ferric oxide form into the ferrous-ferric oxide form, and then by reoxidizing the mass or converting it from the ferrous-ferric oxide form into the ferric form.

10. The process of preparing pulverous iron ores and the like for smelting in blast furnaces, or use in open hearth furnaces,

consisting in first sintering the material, converting the iron oxides contained therein into a ferrous-ferric condition, and then restoring the resulting ferrous-ferric oxides to a ferric condition by exposing the treated material while hot to a current of air.

11. The process of preparing pulverous iron ores and the like for smelting in blast furnaces or use in open hearth furnaces, said process consisting in first continuously feeding the material to be treated into a heating chamber, sintering the exposed surface of the mass of material, heaving the accumulating mass of material, breaking its sintered crust and exposing its unsintered portions to the heat in said chamber until sintered, and then exposing the broken crust while hot to a current of air bringing it to a ferric condition.

12. The process of preparing pulverous iron ores and the like for smelting in blast furnaces or use in open hearth furnaces, consisting in continuously feeding the material to be treated into a heating chamber, and exposing the surface of the mass of material to a sufficient heat to form thereon a sintered crust, heaving the mass of material sufficiently to break its sintered crust and turn the same so as to expose its unsintered parts to the reflected heat in said chamber, and then depositing the sintered material at a point where it is exposed to a current of air passing into said heating chamber whereby said material may be simultaneously cooled and restored to a ferric condition.

SIDNEY CORNELL.

Witnesses:

W. E. REED,  
H. L. BLACK.